

# UNITED STATES PATENT OFFICE.

WOODBRIDGE H. BIRCHMORE, OF BROOKLYN, NEW YORK, ASSIGNOR OF  
ONE-HALF TO CLARKSON A. COLLINS, OF NEW YORK, N. Y.

## PROCESS OF MAKING INCANDESCING MANTLES.

SPECIFICATION forming part of Letters Patent No. 684,493, dated October 15, 1901.

Application filed March 14, 1900. Serial No. 8,661. (No specimens.)

*To all whom it may concern:*

Be it known that I, WOODBRIDGE H. BIRCHMORE, a citizen of the United States, residing in the borough of Brooklyn, city of New York, county of Kings, in the State of New York, have invented a new and Improved Process of Making Incandescing Mantles, of which the following is a specification:

My invention relates to that class of mantles used for the purpose of illumination which become incandescent when subjected to a heating-flame. Such mantles have heretofore been made by saturating a suitable combustible fabric with a solution of those metallic earth oxids which when heated become highly incandescent, from which the fabric is then burned out, leaving a skeleton consisting entirely of the metallic earth oxids. Such mantles are extremely fragile and are expensive to make on account of the high cost of the materials employed.

To the end of obviating these objections and producing mantles of greater rigidity and durability at less cost my invention broadly consists in making an incombustible mantle base, form, or skeleton which may be only slightly incandescent when heated, but which shall be relatively rigid and durable and which may be made of inexpensive materials, and then giving to such form a thin coating of the metallic earth oxids, whereby all their light-giving power is attained for the mantle by the use of the smallest possible amount of material. In order to accomplish this, I take any suitable combustible fabric, such as the usual well-known mantle material woven of cotton, which, either before or after being saturated, as hereinbefore described, is formed into mantles of any usual or desired shape and size. The mantle material I saturate with a solution formed by adding oxid of magnesium to a solution of oxid of zinc dissolved in hydrochloric acid until the solution is practically neutral and diluted with water until thin enough to thoroughly penetrate and fill the pores of the fabric. The mantle fabric thus saturated having been given the shape which the mantles are to have is thoroughly

dried and then exposed to a hot highly-oxygenated flame until the woven fabric of the 50 mantle is entirely burned out and the metallic salts are completely oxidized, the completion of this step being indicated by the mantle becoming incandescent. The mantles thus formed I then treat after cooling with a dilute solution of a mixture of the metallic earth oxids, which become incandescent when heated, such as has heretofore been used in making incandescent mantles, as is well known in the art, so as to cover the mantle 55 with a thin coating of such solution. Preferably I apply this solution to the mantles in a fine spray; but any other suitable method of application by which the desired thin coating can be obtained may be employed. The mantles are then ready for use. The incombustible mantle form or base formed from the oxychlorid of zinc and oxid of magnesium is much more rigid and durable than the mantles heretofore known, and the coating of the 60 metallic earth oxids applied to this base gives to the mantle the same light-giving power possessed by those composed entirely thereof.

I am thus enabled to produce by means of my invention a rigid durable mantle of great 75 illuminating power at an extremely low cost, since the materials of which the base is composed are inexpensive and the amount of the expensive metallic earth oxids required is reduced to a minimum.

What I claim as new, and desire to secure by Letters Patent, is—

The process of making incandescing mantles which consists in saturating a combustible fabric with a solution of oxid of magnesium in oxychlorid of zinc, burning out the combustible fabric therefrom and coating the mantle-form thus made with a solution of metallic earth oxids.

In testimony whereof I have hereunto subscribed my name this 13th day of March, A. D. 1900.

WOODBRIDGE H. BIRCHMORE.

Witnesses:

CHAS. METZ,  
CLARKSON A. COLLINS.